

# UNITED STATES PATENT OFFICE.

ISIDOR KITSEE, OF PHILADELPHIA, PENNSYLVANIA.

## VEGETABLE DYE AND METHOD OF PREPARING THE SAME.

1,254,914.

Specification of Letters Patent. Patented Jan. 29, 1918.

No Drawing.

Application file November 26, 1915. Serial No. 63,367.

To all whom it may concern:

Be it known that I, ISIDOR KITSEE, a citizen of the United States, residing at Philadelphia, county of Philadelphia, and State of Pennsylvania, have invented a new and useful Improvement in Vegetable Dyes and Methods of Preparing the Same, of which the following is a full, clear, and exact description.

My invention relates to logwood or like vegetable dyes. The object of the invention is to produce a vegetable dye by the use of which yarns and textile goods generally may be dyed in various colors and in what are known as "fast" colors.

I have discovered that by the addition to a logwood or other vegetable dye (preferably a purified dye) of two metallic compounds, one at least of which carries an alkali, different shades of black, blue, brown, yellow and red may be obtained, and that the color will remain practically unchanged, that is, "fast" in washing.

The different shades and colors may be varied by varying the proportions of the two compounds relatively to each other and to the logwood dye solution and also by varying the metal base.

The following examples may be given of practicable ways of carrying out my improved process.

If it is desired to dye goods black: To 100 parts by weight of a logwood dye solution (which preferably is purified by the addition thereto of from 1 to 10 parts of sulfuric acid in accordance with my pending application Serial No. 59,759, filed November 5, 1915) are added 3 parts of a concentrated solution of chlorid of zinc and 5 parts of a concentrated solution of copper ammonium chlorid. The chlorid of zinc may be added to the dye solution at any time after the latter is prepared, but the copper ammonium chlorid should not be added until just before it is desired to dye the goods. The process may be carried out at ordinary temperatures. After the goods are dyed, they may be developed in bichromate and nitrate of potassium, or in any other suitable developing substance, for the purpose and in the manner well known in the art; this step forming no part of my invention.

To dye goods blue, the following example may be given:

Dye solution, 100 parts.

Chlorid of zinc (concentrated solution), 3 parts.

Copper ammonium chlorid (concentrated solution), 6 parts.

The dyed goods should preferably be developed in sulfate of copper.

If, for a chlorid of zinc, a chlorid of tin be substituted, a red color may be produced. To produce a brown color, hydrochloric acid may be added.

A person versed in the art will have no difficulty in determining what compounds and what proportions are adapted to produce the particular shades desired. Broadly speaking, it may be stated that the greater the proportion of the zinc salt, the darker the shade of black, and the greater the proportion of ammoniated copper, the lighter the shade of blue.

Having now fully described my invention, what I claim and desire to protect my Letters Patent is:

1. The method of producing fast dyes which consists in adding to a vegetable base, chlorids of two different metals, one of said metals being combined also with an alkali.

2. The method of producing fast dyes which consists in adding to a vegetable base a metallic chlorid and a metallic ammonium chlorid.

3. The method of producing fast dyes which consists in adding to a vegetable base, chlorid of zinc and ammonium copper chlorid.

4. As a new composition of matter, a dye comprising a vegetable base, and chlorids of two different metals one of which is combined with an alkali.

5. As a new composition of matter, a dye comprising a vegetable base, a metallic chlorid and a metallic ammonium chlorid.

6. As a new composition of matter, a dye comprising a vegetable base, chlorid of zinc and ammonium copper chlorid.

In testimony of which invention I have hereunto set my hand at Philada., on this 23<sup>rd</sup> day of Nov., 1915.

ISIDOR KITSEE.

Witness:

JOHN J. RUTHERFORD.